

## UNITED STATES PATENT OFFICE.

ALFRED A. DENNIS, OF GRAND RAPIDS, MICHIGAN.

## METHOD OF TREATING VENEERS.

No Drawing.

Application filed April 6, 1925. Serial No. 21,812.

This invention relates to a method of treating and laying veneers. In the manufacture of furniture of various types it is common to overlay an inner bed with a thin layer of a different and more expensive kind of wood than that from which the bed is made. For instance, in the manufacture of a table top the bed may be of a relatively thick and heavy cheap wood while upon this bed a veneer of much more expensive wood may be laid and glued in place as well as at the side and end edges thereof, the veneer being of a wood capable of receiving a very high finish and one which will present a very attractive appearance when finished.

The veneers used are cut in very thin sheets and in many cases, particularly veneers known as crotch veneers (and the same is true of many other types of so-called hard veneers) such veneers are liable to crack or fracture in handling and particularly after having been applied to the bed or stock which serves as a support therefor, due to the shrinking of the veneer with a consequent formation of checks and cracks therein. This does not occur many times until after the article of furniture to which the veneer has been applied has been out in use for a considerable time but it is well known that checked and cracked veneers on articles of furniture are very common, particularly in household furniture.

It is a primary object and purpose of the present invention to provide a veneer and to treat it that after it is once laid it is not thereafter capable of any shrinkage and, accordingly, is incapable of having checks or cracks produced therein, the veneer before it is laid being shrunk to its absolute minimum and irrespective of any tendency thereafter for the same to enlarge or swell and shrink thereafter it cannot shrink to a point such that checking or cracking of the veneer will ever take place. Articles of furniture having veneers produced according to my method are accordingly insured against any future deterioration from this cause.

In the method of treating and laying crotch or other hard veneers which I have devised, the thin sheets of veneer, single-ply, which have been cut in the usual way are first flattened and straightened, the same being sprayed or dampened with a dressing or sizing so as to moisten the same, the ve-

neers afterward being placed between dry panels or cauls to dry them out and flatten in the usual way, being allowed to remain in this condition over night. The succeeding day the veneer sheets may be dried out between cauls which are but slightly heated at first or lukewarm. The veneers have this process of drying repeated as many times as may be necessary with the cauls heated to higher degrees of temperature until the same are dried so as to eliminate substantially all moisture coming from the application of the dressing or sizing thereto and are ready to be jointed in the usual way if it is necessary for the size of the bed to be covered. The jointing of pieces of veneer is old and well known and need not be entered into at this time other than to say that for any particular piece or pieces of work a sufficiently large sheet of veneer is made by jointing together a plurality of pieces edge to edge to cover the particular piece or pieces of work desired.

When the veneers have been properly jointed and otherwise fixed up to cover the work for which it is designed each is glued to an under veneer preferably of birch or maple. Slightly curly maple veneer is preferred though this is not essential. The veneer first treated is known as face veneer and this is glued to the under-ply of birch, maple or other desired veneer and in applying the face veneer to the under-ply the grain of the under-ply veneer should be parallel to the grain in the face veneer as much as possible; also the joints of the face and under veneers should not lie one over the other but should be separated some distance from each other, it being desirable to always break the joints where the joints are in the same direction.

The thickness of the under veneer preferably is one thirty second of an inch where birch or maple is used, though this may be subject to slight changes of dimensions so far as thickness is concerned. The under and face veneers are glued together in any suitable manner, vegetable glue being used as the same is not subject to crystallization and loss of binding power from heating as animal glue is.

The two-ply veneers made up each of an under-ply of birch or maple preferably, and a face veneer of the selected veneer such as mahogany, walnut or the like having been glued together, have become swollen and ex-

panded due to the moisture absorbed from the glue. The ordinary practice with veneers of this character is to dry the same out by air drying for a period of time, approximately lasting for twenty-four hours and then dry out further either once or twice in heated cauls whereby nearly all of the moisture in the veneers is driven off. This drying is not a rapid process as too rapid a drying may result in causing blisters in the glue line between the veneers, but after a period of air drying followed by some artificial drying in cauls the temperature which will not at the highest likely exceed 125 degrees Fahrenheit, these veneers have heretofore been considered ready for laying on the work, that is, gluing to the articles of furniture with which they are to be used.

With my process and method the veneers at this stage are further subjected to what I consider the essential and necessary step in order to make the same absolutely proof against any checking or cracking after the same have been laid on the work. This step consists in redrying the two-ply veneers taking them at the stage where heretofore they have been considered ready for laying on the work and placing them in what is known as a veneer dryer. The two-ply veneers are placed between the plates of the veneer dryer, the plates closed and let stand for substantially one minute or a little longer but not to exceed two minutes. The temperature of the plates in the veneer dryer may range anywhere between 230 to 300 degrees Fahrenheit but in practice I have found that 260 degrees Fahrenheit gives very satisfactory results. After the plates have been closed for between one and two minutes and the two-ply veneer thus subjected to redrying for that time the plates are opened for a short period to permit any contraction of the two-ply veneer therein, then the plates again closed and let stand for approximately one more minute. The plates are then opened and the veneer taken therefrom, laid in a pile and weighted down so as to keep them as flat as possible.

This completes the operation of redrying the veneers and unless the same are to be laid on the work immediately they must be kept in an absolutely dry place until they are wanted for gluing onto the regular stock therefor.

As a result of the redrying at the high degree of temperature noted all of the moisture is completely expelled from the two-ply veneers and the same has shrunk to its minimum size and can shrink no farther in this state when glued to the under bed or regular stock with which it is used. And the thoroughly dried and completely shrunk two-ply veneer which is laid on the bed cannot expand on account of moisture from the glue used, as this moisture will not penetrate

the super-dried glue line between the face and under-ply veneer so as to reach the face veneer and cause its expansion before the two-ply veneer has been completely and thoroughly bound to the under bed, there being a super-dried glue line between the face and under-ply of the two-ply veneer through which the moisture does not penetrate. Accordingly there can be no further tendency for the veneers to ever further shrink or contract and thus develop checks or cracks therein. There may be tendencies for the veneers to expand but this is counteracted and held against by the absolute tie made between the veneers and the bed to which it is glued and while there may be a potential force of expansion present in the veneers it is held against actively expanding while any drying out of the articles of furniture after they have reached the households where they are to be used cannot dry and contract the veneers below the point to which they were taken by the redrying of this method. No veneer subjected to the method described will thereafter develop any checks or cracks because of shrinking as it has had its greatest possible shrinkage before laying in place and is at its greatest state of shrinkage when it is laid.

This invention while of simple character has proved exceptionally practical in service and is now in use to a large extent.

I claim:

1. The method of treating veneers which consists in gluing together a commercially dry face and backing veneer, drying the same, and then subjecting the same to a redrying operation to thereby completely contract and shrink said veneers to a point beyond which they cannot further shrink, substantially as described.

2. The method of treating veneers which consists in gluing together a commercially dry face veneer and a commercially dry backing veneer, drying the same, and then subjecting the dried two-ply veneer to heat at a temperature between 230 and 300 degrees Fahrenheit to thereby drive off all moisture and completely contract and shrink said veneer to a point beyond which it cannot further shrink, substantially as described.

3. The method of treating veneers which consists in gluing two commercially dry veneers together, then drying the same, and then subjecting the same to superheat at a temperature exceeding the usual highest temperature for drying to thereby drive off all moisture and shrink the veneers to a point beyond which they cannot further shrink, substantially as and for the purposes described.

4. The method of treating veneers which consists in gluing a plurality of commercially dry sheets of veneer together, drying the

- same in accordance with usual practice and then subjecting the same to a redrying operation at a higher degree of temperature to remove all moisture and shrink the veneers to a point beyond which they cannot further shrink, substantially as and for the purposes described.
5. The method of treating veneers which consists in gluing two commercially dry 10 single-ply veneer sheets together, drying the same after gluing in the usual manner, and then subjecting the same for short periods of time to a much higher degree of temperature to completely exclude all moisture and 15 shrink said veneers to a point beyond which they cannot further shrink, substantially as described.
6. The method of treating veneers which consists in gluing together two sheets of 20 commercially dry single-ply veneer, drying the same and then redrying the veneers by subjecting to a temperature between 230 and 300 degrees Fahrenheit for a short period of time and then again subjecting them to said 25 temperature for a second short period of time, substantially as described.
7. The method of treating veneers which consists in gluing together two sheets of commercially dry single-ply veneer, drying 30 the same then clamping the same between heated plates heated to a temperature be-
- tween 230 and 300 degrees Fahrenheit for a short period of time, not exceeding two minutes, then releasing the veneers from the clamping plates and then again clamping 35 the veneers between the plates and subjecting them to said heat for a second short period of time approximating one minute.
8. The method of treating veneers which consists in applying a glue size to two sheets 40 of single-ply commercially dry veneer, drying the same, gluing the two sheets of veneers together, drying the veneer after gluing and then subjecting the ply veneer to high temperature and heat to redry the 45 same and eliminate all moisture from said veneers, and completely shrinking the same to a point beyond which it cannot further shrink, substantially as described.
9. The method of treating veneers which 50 consists in gluing together two thin sheets of commercially dry single-ply veneer, drying the same in accordance with usual practice and then subjecting the same to excess temperature and heat to redry the same and 55 shrink the same to a point beyond which they cannot further shrink, substantially as described.

In testimony whereof I affix my signature.

ALFRED A. DENNIS.